

## UNITED STATES PATENT OFFICE

1,949,588

## COMPOSITION FOR REMOVING CARBON DEPOSITS

Charles A. Thomas and Carroll A. Hochwalt,  
Dayton, Ohio, assignors to Thomas & Hochwalt  
Laboratories, Inc., Dayton, Ohio, a corporation  
of Ohio

No Drawing. Application July 18, 1930, Serial  
No. 468,990

12 Claims. (Cl. 87—5)

This invention relates to compounds for removing carbon deposits such as are formed in internal combustion engine cylinders.

One of the principal objects of this invention is to provide a superior composition which is unusually effective in removing such deposits.

Another object of this invention is to provide such a composition for removing carbon deposits which is quite cheap, and which has no objectionable deleterious effects upon metal parts with which it comes in contact.

Other objects and advantages of the invention will be apparent from the following description and appended claims.

Carbon deposits such as are formed in internal combustion engines are found to consist primarily of the following ingredients:

(1) Road dust, which consists principally of silica; (2) lubricating oil resulting from seepage past the piston rings; (3) graphitic carbon which results primarily from cracking of the gasoline and lubricating oil; and (4) oxidized lubricating oil which results from the oxidation of the ordinary lubricating oil which has seeped past the piston rings, this oil being oxidized at the high temperatures present in the cylinder and in the presence of oxygen of the fuel mixture. The oxidized lubricating oil, which comprises a number of complex and undetermined compounds of carbon, hydrogen and oxygen, forms a resistant binder or cement which binds the road dust and graphitic carbon together to hold them tightly onto the cylinder head, the piston top, and other portions confining the combustion space.

Various solvents, such as alcohol and benzol, which for purpose of description are hereinafter termed, "low boiling organic solvents", have been used in an attempt to dissolve out such deposits. These solvents are found to have a solvent action

upon the ordinary unoxidized lubricating oil but the oxidized lubricating oil or binder is very resistant and is only dissolved to an ineffectual degree by such solvent.

We have discovered that certain compounds, namely the halogenated ethers, have a solvent action upon this binder. For example, the halogenated ethers, having the empirical formula  $C_nH_{(2n+2-x)}R_xO$ , in which R represents a halogen, and x represents the number of substituted halogen atoms, are very effective carbon removers. Thus beta-beta dichlor-ethyl ether,



which is ethyl ether containing two substituted chlorine atoms, is an excellent compound of this

character. We have found that other ethers of this series containing a substituted halogen, such as dichlor-propyl ether,  $C_6H_{12}Cl_2O$ ; and dichlor-butyl ether  $C_8H_{16}Cl_2O$ ; are satisfactory carbon removing compounds in accordance with this invention.

Beta-beta dichlor-ethyl ether is a water white liquid, having a boiling point of 178°C., sp. g. @ 20° of 1.213 and viscosity somewhat higher than that of water. We have found this compound to be especially effective as a solvent for carbon deposits and in removing such deposits from engine cylinders.

In order to insure easy starting of an internal combustion engine after application of the carbon remover, a quantity of a highly volatile combustible is preferably incorporated in the composition. High test gasoline functions very satisfactorily for this purpose.

An effective composition for removing carbon from engine cylinders may be prepared by using a mixture of beta-beta-dichlor-ethyl ether with gasoline in the proportion of about 20% gasoline to 80% beta-beta-dichlor-ethyl ether.

While low boiling organic solvents, such as alcohol and benzol are relatively ineffective when used alone to remove carbon deposits such as are formed in engine cylinders, it has been found that a combination of such solvents with a material having more effective solvent action on the binder, produces a very effective carbon removing composition. Such low boiling organic solvents dissolve any unoxidized lubricating oil in the deposit, and the more difficultly soluble part of the binder is thus brought in direct contact with the more active solvent.

An effective carbon removing composition including such low boiling solvents is prepared as follows:

|                                    | Percent<br>by weight |
|------------------------------------|----------------------|
| High test gasoline.....            | 25                   |
| Denatured ethyl alcohol.....       | 25                   |
| Benzol.....                        | 25                   |
| Beta-beta dichlor-ethyl ether..... | 100                  |

Another very effective composition for removing carbon deposits may be prepared without the use of gasoline, as follows:

|                                    | Percent<br>by weight |
|------------------------------------|----------------------|
| Beta-beta dichlor-ethyl ether..... | 50                   |
| Denatured ethyl alcohol.....       | 25                   |
| Benzol.....                        | 25                   |

In using this composition to remove carbon de-

posit from an internal combustion engine, the engine is first run until it is quite hot. Then the carbon remover is introduced into the cylinder, either by pouring through the intake manifold, care being taken to prevent escape of the solvent through the exhaust ports. Generally from about 20 to 50 c.c. are added per cylinder. The motor is then allowed to stand for some time, preferably about 6 hours or over night, during which time 10 the composition acts upon the binder and renders the insoluble carbon and road dust free and flaky. The motor is then started and allowed to run a short time, the blast serving to blow the loosened solid material out through the exhaust.

15 It is found that the action of this carbon remover is so effective that carbon deposits on engine cylinders may be loosened to such a degree that objectionable knocking of the motor may result, due to the loosened deposits being jammed 20 between the piston and valves and the cylinder head when the motor is again started. This is accentuated in certain types of high compression heads having irregular shape combustion chamber in which the clearance between the piston 25 and head and the valves and the head is quite small at certain points or at one side thereof. With such a high compression head, it is found that loosened carbon deposits may accumulate on the side having small clearance, when these loosened deposits are in a dry condition, and the movement of the piston and the valves during 30 operation jams these deposits against the head with the result that a heavy knocking is produced, which in some instances may even be so 35 serious as to result in cracking of the piston or the head.

We have discovered that this knocking upon restarting of the engine after application of the carbon remover may be overcome by incorporating 40 in the carbon remover a material having a high boiling point so that it is normally liquid at the high temperatures present in the engine cylinders, and which serves to keep the loosened carbon in a wet condition. We have found that 45 such a heat resisting material serves to keep the carbon deposits in a mushy state and the objectionable knocking above referred to is eliminated, although the carbon deposit is effectively discharged through the exhaust when the motor is 50 started. An effective compound of this character is a low melting paraffin, or paraffin oil, which does not readily evaporate at the high temperatures present within engine cylinders and is normally a liquid at these temperatures. Other 55 high boiling compounds such as high boiling oils, or high boiling hydro-carbons such as naphthalene, function satisfactorily for this purpose. Such compounds also add lubricating properties, such that after use of the carbon remover the 60 danger of the piston binding because of solution of the lubricating oil on the cylinder wall is minimized. High boiling chlorinated naphthalenes, such as mono-chlor-naphthalene, di-chlor-naphthalenes and tri-chlor-naphthalenes 65 may be used for this purpose. Di-chlorbenzene is also satisfactory. These halogenated hydrocarbon materials are especially satisfactory because they withstand the heat of the motor without breaking down, and are also in themselves highly efficient carbon removers. Reference is herein made to the co-pending application of Charles A. Thomas and Carroll A. Hochwalt, Serial No. 397,144, filed October 3, 1929, which discloses and claims these halogenated hydrocarbons as carbon removers.

Many carbon removers are solids or semi-solids at ordinary temperatures. In order to make their application easy and effective, such compounds are dissolved in suitable solvents. Low boiling organic solvents such as the various alcohols, ether, acetone, ethyl acetate, kerosene, gasoline, benzene and the like, have usually been used, but these are in themselves ineffectual solvents of carbonaceous resinous deposits. Beta-beta-dichlor-ethyl ether, being itself a liquid at ordinary temperatures and having high solvent properties may be used very effectively as a carbon remover without the usual low boiling organic solvents.

As an example of a superior and preferable 90 composition incorporating high test gasoline and a high boiling material to prevent knocking, the following may be used:

|                               | Per cent by weight | 95  |
|-------------------------------|--------------------|-----|
| High test gasoline            | 20                 |     |
| Denatured ethyl alcohol       | 20                 |     |
| Benzol                        | 20                 |     |
| Mono-chlor-naphthalene        | 20                 | 100 |
| Beta-beta-dichlor-ethyl ether | 20                 |     |

While the compositions herein described constitute preferred embodiments of the invention, it is to be understood that the invention is not limited to these precise compositions and that 105 changes may be made therein without departing from the scope of the invention which is defined in the appended claims.

What is claimed is:

1. A composition for removing carbon deposits 110 from engine cylinders comprising beta-beta<sup>1</sup> dichlor-diethyl ether, denatured ethyl alcohol and benzol.

2. A composition for removing carbon deposits 115 from engine cylinders comprising beta-beta<sup>1</sup> dichlor-diethyl ether, denatured ethyl alcohol, mono-chlor-naphthalene, benzol and high test gasoline.

3. A composition for removing carbon deposits 120 from engine cylinders comprising a mixture of a low boiling organic solvent for lubricating oils with more than 10% by weight of a halogenated ether of the empirical formula  $C_nH_{(2n+2-x)}R_xO$ , where R represents a halogen, and x the number of substituted halogen atoms in the molecule. 125

4. A composition for removing carbon deposits from engine cylinders comprising as an essential ingredient a halogenated ether of the empirical formula  $C_nH_{(2n+2-x)}R_xO$ , where R represents a halogen, and x the number of substituted halogen atoms in the molecule. 130

5. A composition for removing carbon deposits from engine cylinders comprising as an essential ingredient a chlorinated ether of the empirical formula  $C_nH_{(2n+2-x)}Cl_xO$ , where x represents the 135 number of substituted chlorine atoms in the molecule.

6. A composition for removing carbon deposits from engine cylinders comprising a mixture of a low boiling organic solvent for partially oxidized lubricating oils with a chlorinated ether of the empirical formula  $C_nH_{(2n+2-x)}Cl_xO$ , where x represents the number of substituted chlorine atoms in the molecule. 140

7. A composition for removing carbon deposits 145 from engine cylinders comprising a mixture of a low boiling organic solvent for partially oxidized lubricating oils with beta-beta<sup>1</sup> dichlor-diethyl ether.

8. A composition for removing carbon deposits 150

from engine cylinders comprising a high boiling point material of the group consisting of paraffin and paraffin oils, mixed with a chlorinated ether of the empirical formula  $C_nH_{(2n+2-x)}Cl_xO$ , where 5  $x$  represents the number of substituted chlorine atoms in the molecule.

9. A composition for removing carbon deposits from engine cylinders comprising a halogenated naphthalene, and a halogenated ether of the empirical formula  $C_nH_{(2n+2-x)}RxO$ , where  $R$  represents a halogen, and  $x$  the number of substituted halogen atoms in the molecule.

10. A composition for removing carbon deposits from engine cylinders comprising a halogenated benzene, and a halogenated ether of the empirical formula  $C_nH_{(2n+2-x)}RxO$ , where  $R$  represents

a halogen, and  $x$  the number of substituted halogen atoms in the molecule.

11. A composition for removing carbon deposits from engine cylinders comprising a chlorinated naphthalene, and a chlorinated ether of the empirical formula  $C_nH_{(2n+2-x)}Cl_xO$ , where  $x$  represents the number of substituted chlorine atoms in the molecule. 80

12. A composition for removing carbon deposits from engine cylinders comprising a chlorinated benzene, and a chlorinated ether of the empirical formula  $C_nH_{(2n+2-x)}Cl_xO$ , where  $x$  represents the number of substituted chlorine atoms in the molecule. 85

CHARLES A. THOMAS. 90  
CARROLL A. HOCHWALT. 95

20 95

25 100

30 105

35 110

40 115

45 120

50 125

55 130

60 135

65 140

70 145

75 150